

# United States Patent [19]

Flesher et al.

[11] Patent Number: 4,859,720

[45] Date of Patent: Aug. 22, 1989

[54] PROCESS AND COMPOSITIONS FOR SIZING PAPER

[75] Inventors: Peter Flesher; John Langley; Norma Rosier; David Farrar, all of West Yorkshire, England

[73] Assignee: Allied Colloids Ltd., England

[21] Appl. No.: 11,062

[22] Filed: Feb. 4, 1987

Related U.S. Application Data

[63] Continuation-in-part of Ser. No. 857,115, Apr. 29, 1986, abandoned, and a continuation-in-part of Ser. No. 667,950, Nov. 5, 1984, abandoned.

[30] Foreign Application Priority Data

Nov. 7, 1983 [GB] United Kingdom ..... 8329655  
May 3, 1985 [GB] United Kingdom ..... 8511379

[51] Int. Cl. 4 ..... C08J 3/00

[52] U.S. Cl. ..... 523/332; 524/112

[58] Field of Search ..... 524/112; 523/332

[56] References Cited

U.S. PATENT DOCUMENTS

4,207,142 6/1980 Shepherd ..... 162/158  
4,214,948 7/1980 Mazzarella et al. ..... 162/158  
4,279,794 7/1981 Dumas ..... 524/112  
4,431,826 2/1984 Sweeney ..... 162/158 X

4,514,229 4/1985 Sato et al. ..... 524/112 X  
4,545,855 10/1985 Sweeney ..... 162/158  
4,645,568 2/1987 Kurps et al. ..... 523/332

FOREIGN PATENT DOCUMENTS

2439026 2/1975 Fed. Rep. of Germany ..... 162/158  
0045730 3/1983 Japan ..... 524/112  
0045731 3/1983 Japan ..... 524/112

Primary Examiner—Joseph L. Schofer

Assistant Examiner—J. M. Reddick

Attorney, Agent, or Firm—Ostrolenk, Faber, Gerb & Soffen

[57]

ABSTRACT

A concentrate composition, that can be diluted with water to form an aqueous size for cellulosic fibres, comprises a substantially anhydrous dispersion of polyelectrolyte particles in a non-aqueous liquid comprising a reactive size, and is made by forming a dispersion in a hydrophobic liquid of the polyelectrolyte particles while they are swollen by water, azeotroping the dispersion and adding the size to the hydrophobic liquid. If the size is a liquid size, the hydrophobic liquid may be removed from the composition. The dispersion of swollen polyelectrolyte particles in the hydrophobic liquid can be made by dispersing a solution of polyelectrolyte in the liquid but is preferably made by reverse phase polymerization.

17 Claims, No Drawings

PROCESS AND COMPOSITIONS FOR SIZING  
PAPER

This application is a continuation-in-part of U.S. Ser. No. 667,950 filed Nov. 5, 1984 and a c-i-p of U.S. Ser. No. 857,115 filed Apr. 29, 1986, both now abandoned.

The invention relates to the sizing of cellulosic fibres and to compositions for use in this, and to their manufacture.

During the manufacture of paper it is necessary to render the naturally hydrophilic cellulosic fibres hydrophobic so that penetration of aqueous liquids into the formed sheets is limited thereby making writing and printing on the sheets possible. This process, known as sizing, can be carried out by adding a sizing agent to the pulp slurry (usually termed internal sizing) or the sizing agent can be applied to the formed paper sheet. This invention is concerned with the internal sizing process.

There are two types of sizing agent in general use. One of these is based on rosin which is used in conjunction with alum. The rosin is added as a soap solution or as an emulsion and alum is added afterwards just prior to sheet formation to precipitate the rosin as a fine particulate which is retained by the sheet.

The second type of size is a reactive size, such as a ketene dimer or an anhydride-based size, which reacts chemically with the cellulosic fibres. Preferably it is applied in combination with a polyelectrolyte which will help to retain the size in the sheet.

The reactive size is generally added to the pulp in the form of an aqueous emulsion, generally a cationic emulsion. The emulsion can be prepared at the mill but this necessitates the mill having emulsifying equipment and so it would be more convenient if a concentrated emulsion could be supplied to the mill ready for dilution and use. Unfortunately, reactive sizes tend to react with water so that an aqueous emulsion is liable to be rather unstable.

Anhydride based sizes, such as alkenyl succinic anhydride sizes, are so reactive that their emulsions have to be prepared at the mill just prior to use. These sizes are normally supplied to the mill with a cationic starch which generally has to be precooked before emulsification, thus making it even less convenient for the emulsion to be formed at the mill.

Ketene dimer sizes often are supplied to the mill in the form of an emulsion but these emulsions have only limited shelf-life and the maximum concentration of ketene dimer in the emulsion is rather low, generally below 6%, so that very large volumes of emulsion have to be supplied to the paper manufacture.

Emulsification of liquid ketene dimers can be achieved using conventional emulsification equipment but some of the preferred ketene dimers are solids at ambient temperature. As described in U.S. Pat. No. 3,046,186, emulsification of these necessitates initially either melting the solid (so that upon cooling the emulsion is converted to a dispersion) or dissolving the solid in a solvent, generally benzene. A typical important ketene dimer is distearyl ketene dimer and this has only relatively low solubility in organic solvents with the result that the solution of it that is emulsified must be rather dilute. For instance, we have found that this dimer precipitates from a 40% by weight solution in benzene (weight ratio benzene:dimer of 1:0.67) and so any solution in benzene must be much more dilute than

this. Also this dimer is less soluble in other organic solvents than it is in benzene.

As described in U.S. Pat. No. 3,046,186, the emulsions are generally prepared by emulsifying the dimer into an aqueous solution of cationic dispersing agent although that patent does mention that in certain instances the emulsifying agent may be predispersed in the ketene dimer. It is stated that the emulsions may be prepared at any convenient solids content but are used 10 at 1 to 5% solids by weight.

In each of the examples in U.S. Pat. No. 3,046,186, the initial composition that was prepared and that contained both size and polyelectrolyte was very dilute. For instance in Example 1 the initial concentration is 15 about 9% by weight size based on the total composition.

As mentioned above, it is preferred to provide a polyelectrolyte with the reactive size and it might be thought that some of the disadvantages associated with providing emulsions of reactive size and polyelectrolyte 20 could be minimised if the reactive size and the polyelectrolyte were supplied separately. However this incurs other disadvantages.

It would therefore be very desirable if it was possible to supply a stable concentrated composition that contained both reactive size and polyelectrolyte and which was readily dilutable with water at the mill.

A concentrate composition according to the invention comprises a substantially anhydrous dispersion of a polyelectrolyte in a non-aqueous liquid comprising a 30 reactive size. If the reactive size is liquid, the non-aqueous liquid may consist of the size, in the substantial absence of solvent. Often, however, the non-aqueous liquid is a solution of the size in a hydrophobic liquid. The composition is best made by dissolving the reactive 35 size in a substantially anhydrous dispersion of the polyelectrolyte in a hydrophobic liquid. The dispersion is best made by reverse phase polymerisation.

The concentrate composition generally has a reactive size concentration above 20% and preferably at least 40 28.6%. The concentration of reactive size is often in the range 30 to 60%. The amount may be higher, for instance up to 80% or 85%. All these amounts are by weight of the total composition.

The weight ratio, on a dry basis, of polyelectrolyte: 45 reactive size is generally from 1:1 to 1:10, preferably 1:1.5 or 2 up to 1:4 or 1:5.

When the liquid phase comprises hydrophobic solvent, in order that the concentrate can conveniently have an appropriately high active content it is necessary for the weight of reactive size to be at least 0.67 part per part by weight organic solvent (i.e. 40% solution). The weight ratio organic solvent:reactive size is generally from 1:10 to 1:0.67 preferably 1:1 to 1:3.

With the most dilute solution of reactive size in solvent that is generally used in the invention (40 parts size to 60 parts solvent), the amount of polyelectrolyte is generally between 4 parts and 40 parts, giving sizing compositions having a reactive size content of from 38.4 to 28.6%. A composition having 83.3% reactive size 55 can be formed from, for instance, 100 parts reactive size, 10 parts solvent and 10 parts polyelectrolyte.

Preferred compositions that contain solvent have, per part solvent, about 1 to 3 parts (preferably about 2 parts) reactive size and about 0.5 to 2 parts (preferably about 1 part) polyelectrolyte.

In the compositions according to the invention that are substantially free of solvent, at least 80%, preferably at least 85% or at least 90%, consists of the polyelectro-

lyte and the liquid size. Preferred compositions contain from 45 to 90%, preferably 60 to 80%, by weight reactive size, 10 to 50%, preferably 20 to 40%, by weight polyelectrolyte and optionally up to 15%, e.g., 5 to 10% additives.

The compositions may contain minor additives such as 0.5 to 5% stabiliser and/or water-in-oil emulsifiers and oil-in-water emulsifier.

The concentrate composition must be substantially anhydrous in order that the composition is stable, and in practice this means that if water is present its amount will be not more than about 5% by weight of the composition. Preferably the water content is not more than about 1% or, at the most, about 2% by weight of the composition. The amount of water is insufficient to form a solution of the polyelectrolyte and preferably is not significantly more than, and most preferably is the same as or less than, the equilibrium moisture content of the polyelectrolyte (i.e. the water content of the electrolyte if it is exposed in the form of dry powder to the ambient atmosphere).

When the liquid phase in which the polyelectrolyte is dispersed is a solution of the reactive size in an organic liquid, this liquid should be a hydrophobic solvent. Suitable solvents are water immiscible organic hydrocarbon liquids such as benzene, xylene, toluene, mineral oils, kerosene, and vegetable oils. In addition to being substantially free of water, the composition is preferably also substantially free of any highly polar liquids with which the reactive size might tend to react. Preferably the liquid phase of the composition consists essentially only of the size and, if desired or necessary, hydrophobic solvent.

When the size is solid, the liquid phase must be a solution of the size in hydrophobic solvent. When the size is liquid, the liquid phase can be provided by the size alone or by a solution of the size in hydrophobic solvent. If the liquid phase is to be provided by the size alone (e.g., below 5%, and usually below 1%, solvent by weight of the composition) the size must be liquid at the temperature at which the composition is used or stored such as 20° to 25° C., and preferably it is liquid at 0° C.

Any type of reactive size may be used in the invention but the size preferably is a ketene dimer reactive size or an anhydride reactive size.

Suitable ketene dimer reactive sizes that may be used include the dimers derived from readily available commercial fatty acids such as palmitic, stearic, oleic or myristic acids or mixtures thereof. Naturally the keten dimer either be a liquid or, more usually, must be soluble in the organic liquid chosen for the polymer-in-oil dispersion. Suitable materials are well known and are described in, for example, U.S. Pat. No. 3,046,186. The ketene dimer may be solid or liquid, but generally the most concentrated products are obtainable when the dimer is liquid.

Suitable anhydride reactive sizes that may be used include alkenyl succinic anhydride sizes. Suitable materials are described in U.S. Pat. No. 3,102,064.

If the composition is to be substantially free of solvent, it is usually preferred for the size to be a liquid anhydride size, although some liquid ketene dimer sizes can be used.

The polyelectrolyte will generally be water soluble and an advantage of the invention is that it can have a any desired molecular weight and in particular can have a molecular weight that is higher than is conveniently

possible with existing compositions. For instance, the intrinsic viscosity can typically be above 1 and generally above 3, e.g., above 6. Although it is generally below 9 it can be higher, e.g., up to 20 or more.

The polyelectrolytes may be cationic or anionic, the cationic polyelectrolytes generally being preferred.

Preferred cationic electrolytes include homopolymers or copolymers of diallyl dialkyl (generally dimethyl) ammonium chloride and homopolymers and copolymers of dialkylaminoalkyl (meth) acrylates and (meth)carylamides (preferably dimethylaminoethyl acrylates and methacrylates) present as acid addition salts or quaternary ammonium salts, generally quaternised with methyl chloride or dimethyl sulphate. Copolymers of such monomers may be formed with acrylamide or methacrylamide and will typically contain at least 10%, and usually at least 30%, by weight of the cationic monomer. Other cationic (meth) acrylamides and other cationic polymers obtained by polymerising one or more ethylenically unsaturated monomers can be used. Other cationic polymers that can be used are polyamines and polyimines such as polyamine-epihalohydrin polymers and dicyandiamide condensates and polyethylene imines.

Suitable anionic polymers include polymers formed from monomers including carboxylic or sulphonic acid groups. These groups may be present as free acid or, more usually, as a water soluble ammonium or alkali metal (generally sodium) salt. Suitable acids are acrylic acid, methacrylic acid and 2-acrylamido-2-methyl-propane sulphonic acid. The anionic polymers may be homopolymers of such acids, or mixtures thereof, or copolymers with, for instance, acrylamide. A suitable polymer is polyacrylamide containing up to 25% or more acrylic acid groups.

The concentrate composition is best made by adding the reactive size to a substantially anhydrous dispersion of a polyelectrolyte in the hydrophobic liquid and thereby forming a solution of the size in the hydrophobic liquid. If the concentrate is to include solvent for the size then the resultant composition can be used without further treatment, although if desired additional hydrophobic liquid can be added and/or some of the hydrophobic liquid can be removed by, for instance, distillation.

If the concentrate is to be substantially free of solvent, then it is necessary to remove the solvent after adding the size and in such processes it is desirable that the solvent used initially as the continuous phase of the dispersion should be a volatile non-aqueous liquid, generally a volatile aliphatic hydrocarbon.

The dispersion of the polyelectrolyte particles in the hydrophobic liquid is best made by forming a dispersion in the hydrophobic liquid of the polyelectrolyte particles swollen by water and then dehydrating this dispersion, generally by azeotroping. This dispersion may be made by dispersing aqueous polymer solution into the hydrophobic liquid in the presence of water-in-oil emulsifier and optionally with other stabiliser, e.g., an amphiphilic polymeric stabiliser. For polymers, e.g., of acrylic monomers, that can be made by reverse phase polymerisation, the dispersion is preferably made by reverse phase polymerisation. Thus an aqueous solution of the monomer or monomers from which the polyelectrolyte is to be formed may be dispersed in an oil phase and then polymerised by emulsion or suspension polymerisation mechanism to form aqueous gel poly-

mer droplets dispersed in the oil phase, and the composition is then dried.

The dry particle size of the dispersion of polyelectrolyte in organic liquid should be typical for reverse phase processes, i.e., below 10  $\mu\text{m}$ , and often below 3  $\mu\text{m}$ . Thus at least 90% by weight should be below 3  $\mu\text{m}$ . Preferably it is below 2  $\mu\text{m}$ , often mainly in the range 0.05 to 1  $\mu\text{m}$ . This very low particles size promotes the formation of a stable dispersion without the need for large amounts of stabiliser. The problems of dusting and mixing, that would be associated with the use of dry powder of this size, are avoided by first forming a dispersion of these particles in organic liquid and then adding the size.

The dispersion is best made by reverse phase polymerisation, generally reverse phase suspension polymerisation, of water soluble monomer or monomer blend dispersed in water immiscible organic liquid.

The reverse phase polymerisation may be conducted in the presence of an oil soluble polymer, generally an amphipathic polymer, as a dispersion stabiliser and this stabiliser may also promote the stability of the final dispersion in the liquid size. The reverse phase polymerisation may also be conducted in the presence of a water in oil emulsifier. Materials and processes for reverse phase polymerisation are well known and are described in, for instance, EP No. 0126528.

It appears that the presence of residues of the described stabilisers on the polymer particles are important for stabilising the concentrates and so even if the concentrate is made by dispersing a solution of polyelectrolyte into the organic liquid, followed by azeotroping, preferably amphipathic polymer is included in that emulsion.

Preferred polymerisation stabilisers are copolymers of one or more hydrophobic ethylenically unsaturated monomers with one or more hydrophilic ethylenically unsaturated monomers. They include polyhydroxy stearic acid-polyethylene glycol condensates, maleic polymers such as those described in U.S. Pat. No. 4,339,371 and, preferably, copolymers of hydrophilic acrylic monomers and hydrophobic acrylic monomers such as those described in GB No. 1,482,515 or EP No. 0126528.

It is particularly advantageous in the invention to use an azeotroped polyelectrolyte dispersion in hydrophobic liquid as the means for supplying the polyelectrolyte, rather than using any other form of polyelectrolyte. If the polyelectrolyte is merely dissolved in aqueous solution and is then blended with the size, a conventional aqueous emulsion will be obtained, rather than the anhydrous concentrates of the invention. If the polyelectrolyte is provided as a powder, the concentrate will generally have a tendency towards settlement upon storage and so either must be used quickly, before serious settlement occurs, or an appropriate dispersion promoter must be added in an effective amount, e.g., 0.01 to 10%. Unlike the amphipathic polymeric stabilisers that are soluble in the oil phase, many of these dispersion promoters are insoluble and typically are clays and other silica based dispersion stabilisers known for stabilising dispersions of particles in oil. However the inclusion of these additional stabilisers is inconvenient, detrimentally affects the viscosity and flow properties of the concentrates, and results in unwanted material being introduced into the aqueous suspension that is sized by the composition.

A user composition is made from the concentrate composition, generally by the user, by adding the concentrate composition to water and thereby forming an oil-in-water emulsion of the size solution dispersed in water in which the polyelectrolyte is dissolved. Formation of the oil-in-water emulsion is promoted by application of mechanical high shear and/or by the presence of an oil-in-water emulsifying agent, such as an ethoxylated nonyl phenol. The oil-in-water emulsifying agent may be included in the concentrate or in the water in which the emulsion is formed.

The water in which the emulsion is formed may be the water of the cellulosic pulp suspension that is to be treated but preferably the concentrate is first converted into an aqueous emulsion to give a reactive size concentration of from 0.01 to 5%, preferably 0.05 to 1%, based on the weight of the aqueous solution.

This emulsion may then be added to the aqueous cellulosic pulp, and paper may be made from it, in the usual way. The amount of reactive size in the aqueous pulp is generally from about 0.01 to about 1% by weight based on the dry weight of the pulp. Upon addition to the pulp slurry, the active size/oil droplets are retained by the polymer on the fibres and the size reacts with the fibres. The size released from an emulsion in this way produces results at least as good as those obtained with the conventional ketene dimer emulsions.

Thus by the invention we obtain sizing results at least as good as those obtained using known compositions and yet for the first time we have the ability of supplying storage stable concentrated compositions that the user can easily convert into aqueous solutions.

The following are examples of the invention.

#### 35 Polyelectrolyte Dispersions

A substantially anhydrous dispersion of a copolymer of methyl chloride quaternised dimethylaminoethyl methacrylate (DMAEMA) and acrylamide was prepared by a reverse phase dispersion polymerisation process. The acrylamide was supplied as a 57% aqueous solution and the quaternised monomer was a 65% aqueous solution. These solutions were dispersed in a blend of Solvent Pale Oil 150 and perchloroethylene in the presence of a polymeric amphipathic stabiliser and a very small amount of emulsifier, in known manner. Polymerisation was initiated and allowed to complete in conventional manner and the resultant product was distilled under reduced pressure to remove the water and the perchloroethylene. The Intrinsic Viscosity of this polymer (and of the polymers in each of Dispersions A to E below) was in the range 4 to 6.

In one process, the ratio DMAEMA:acrylamide was 80:20 by weight and the resultant polymer dispersion, labelled Dispersion A, contained 47.5% by weight of active polymer. A 1% solution of the polymer in water had a RVT Brookfield Viscosity of 6,400 cps at room temperature using spindle No. 3 rotating at 10 rpm.

In another experiment, the monomer proportions were the same and the molecular weight of the resultant polymer was above 106. The resultant dispersion was labelled Dispersion B.

In another process, a dispersion, labelled Dispersion C, was obtained broadly as described for Dispersion A and was a 50% active polymer dispersion in mineral oil.

In another process, the ratio DMAEMA:acrylamide was 30:70 by weight and the resultant dispersion, labelled Dispersion D, contained 50% by weight active

polymer. The polymer in the dispersion was of low molecular weight, having an intrinsic viscosity of 3.16.

In another process, a substantially anhydrous dispersion of a polyamine-epichlorhydrin condensate was prepared by emulsifying the polymer produced in an aqueous phase polymerisation process into a mixture of solvent pale oil 60 and SBP 11 with a very small amount of emulsifiers prior to distilling off the water under reduced pressure. The resultant polymer dispersion, labelled Dispersion E, contained 37.6% by weight of 10 active polymer.

### EXAMPLES 1 to 5

A series of concentrate compositions according to the invention were made by dissolving a reactive size in 15 each of Dispersions A to E.

In Example 1, the size was hexadecenyl dimer and the concentrate contained 1.05 g Dispersion A and 4 g of hexadecenyl ketene dimer, and 1 g of an oil-in-water emulsifier to give a 64.5% active sizing composition. 20 The water content of the concentrate was less than 1%. The product is concentrate A.

In Example 2, the concentrate was made by mixing 2 ml of Dispersion B with 2 ml octadecenyl ketene dimer, to make concentrate B.

In Example 3, one part by weight Dispersion C was mixed with one part by weight alkenyl succinic anhydride reactive size to form concentrate C.

In Example 4, alkenyl succinic anhydride was dissolved into a mixture of Dispersion D and a mineral oil 30 such that concentrate D contained 2 g Dispersion D, 5 g alkenyl succinic anhydride, 2.25 g mineral oil and 0.75 g of an oil-in-water emulsifier to give a 50% active sizing concentrate D, having a water content of less than 1%.

In Example 5, alkenyl succinic anhydride was dissolved into Dispersion E in the presence of emulsifiers to form concentrate E containing 5 g alkenyl succinic anhydride, 5.31 g Dispersion E and 1.28 g of the oil-in-water emulsifiers to give a 43.1% active size concentrate.

Each of concentrates A to E was used to prepare a corresponding aqueous emulsion, having a 1% by weight active size content, by stirring the appropriate amount of dispersion into water. Each of these 45 active emulsions was further diluted to 0.1% by weight active size content and these 0.1% emulsions were labelled Emulsions A to E (having been prepared from, respectively, concentrates A to E).

The effectiveness of each of the emulsions for sizing 50 cellulose fibres was determined by the 1 minute Cobb Test. In each of these tests, hand sheets were prepared on a standard laboratory sheet making machine from a stock containing calcium carbonate and the sheets were then dried and the 1 minute Cobb value determined. 55 For Emulsions A to D, the stock was a bleached sulphate/bleached bird stock but for Emulsion E it was a bleached sulphate (kraft).

In Test A, the hand sheets were 100 g.sm and the stock contained 20% calcium carbonate and was a 0.5% 60 constituted stock. The emulsion was either Emulsion A or, as a comparison, with Emulsion F which was a conventional emulsion prepared from a commercially available 6% emulsion of ketene dimer in water stabilised with cationic starch.

In Test B, hand sheets were prepared from a stock of 50% bleached sulphate, 40% bleached birch and 10% calcium carbonate, beaten to a freeness of 52° S.R. The

stock was sized with Emulsion B or, as a comparison, with Emulsion G obtained by mixing 2 ml of the 50% dispersion of polymer in oil used in the preparation of Dispersion B into 196 mls deionised water followed by rapid stirring with a Silverson mixer at maximum speed and injection into the resultant solution of 2 mls octadecenyl ketene, Silverson mixing being continued for a further 25 seconds. The resultant 1% emulsion was diluted to 0.1% to form Emulsion G.

In Test C, 70 gsm hand sheets were prepared from a stock of 50 parts bleached sulphate, 40 parts bleached birch and 10 parts calcium carbonate and these were sized either with Emulsion C or with comparison Emulsion H. This was prepared as follows. A 12% aqueous dispersion of a cationic starch was cooked at 95° C. for 20 minutes with constant stirring. The cooked starch was cooled and diluted to 9% activity. 2 parts by weight of alkenyl succinic anhydride was added to 3 parts by weight of cationic starch with agitation. High shear mixing using a Silverson mixer was continued to achieve a fine particle size emulsion. This emulsion was diluted with water to 0.75% active size, which was further diluted to 0.1%.

In Test D, 70 gms hand sheets were prepared from a stock of 50 parts bleached sulphate, 40 parts bleached birch and 10 parts calcium carbonate beaten to 50° S.R. and after manufacture, the sheets were placed on glazing plates and pressed at 3.5 kg/cm for 5 minutes prior to drying on rings at 110° C. for 2 hours. Emulsion D was used for sizing each of these sheets.

In Test E, 70 gms hand sheets were prepared from a bleached sulphate stock in conventional manner and dried and pressed as in Test D, the sheets being sized using Emulsion E.

The dosage and the Cobb value are shown in the following Table. The dosage is recorded as percent active size based on dry weight of paper. The Cobb figure is the 1 minute Cobb value.

| Test | Emulsion | Dose | Cobb |
|------|----------|------|------|
| A    | A        | 0.15 | 27.4 |
|      | A        | 0.2  | 25.8 |
|      | F        | 0.15 | 33.2 |
| B    | B        | 0.2  | 26   |
|      | G        | 0.2  | 65   |
| C    | C        | 0.3  | 21.2 |
|      | C        | 0.4  | 19.4 |
|      | H        | 0.3  | 21.6 |
|      | H        | 0.4  | 19.8 |
| D    | D        | 0.2  | 25.6 |
|      | D        | 0.3  | 17.0 |
|      | D        | 0.5  | 14.3 |
| E    | E        | 0.5  | 36.2 |

These results show that the methods and emulsions of the invention, A to E, are all capable of giving satisfactory sizing. Test C shows that the results can be similar to those obtainable with a conventional commercially available 2-pack system H while Test B shows that the results can be surprisingly better than the results obtained by sequential formation of a single emulsion, G. Test A shows that the results can be better than obtainable with a conventional emulsion system. Similarly satisfactory results are obtained when the polymer is polyacrylamide containing 10% molar acrylic acid groups (as sodium salt) and the stock contains alum and has a pH of 5.5.

Additional to these results is the remarkable convenience of the invention to the mill operator in that in-

stead of having to purchase or prepare large volumes of a dilute emulsion, which then have to be stored at the mill, it is possible for the mill operator to purchase or prepare small volumes of a very concentrated emulsion and merely dilute this at the point of use when required.

#### EXAMPLE 6

(Comparative)

A polyelectrolyte, a copolymer of methyl chloride quaternised dimethyl aminoethylmethacrylate and acrylamide (25:75 by weight), was prepared by bulk solution polymerisation. The resulting polymer gel was cut into particles less than 5 mm in dimension, dried on a fluid bed drier and then ground down to the required dimension of less than 53 microns.

A sizing concentrate was prepared, including alkenyl succinic anhydride as the active sizing constituent, by dispersing the powdered polyelectrolyte into the liquid sizing component to which had been added an oil-in-water emulsifying surfactant.

The chosen alkenyl succinic anhydride was a liquid at ambient temperature and did not require melting to allow the dispersion to take place.

The composition comprised 65 g of alkenyl succinic anhydride, 10 g of oil-in-water emulsifying surfactant, and 12.5 g of polyelectrolyte to give a 74.3% active sizing composition. The composition was ostensibly free from water.

It settled rapidly on storage and so had to be used very quickly after manufacture.

2.7 g of the concentrate composition was, quickly after manufacture, added to 197.3 g of water with stirring to give a 1% active alkenyl succinic anhydride emulsion which was used to carry out 1 minute Cobb tests. This emulsion was labelled I.

For this test, 100 gsm handsheets were prepared from a bleached sulphate/bleached birch stock containing 10% calcium carbonate loading, on a Standard Laboratory sheet making machine. Prior to sheet formation, the required amount of 1% alkenyl succinic anhydride emulsion as prepared above was added to 600 mls of 1.0% consistency stock. After stirring, handsheets were prepared on the standard sheet-making machine. The sheets were couched off the sheet-machine in the normal manner placed on glazing plates and pressed at 50 psi for 5 minutes prior to drying on rings at 110° C. for 1 hour. After conditioning at room temperature, the degree of sizing achieved was measured by the standard 1 minute Cobb test. The results are shown in the table below.

| Emulsion | Dose Level of Alkenyl Succinic Anhydride based on Dry Fibre and Filler | 1 Minute Cobb Value (g · m <sup>2</sup> ) |
|----------|------------------------------------------------------------------------|-------------------------------------------|
| I        | 0.23%                                                                  | 18.1                                      |
| I        | 0.34%                                                                  | 15.9                                      |
| I        | 0.57%                                                                  | 13.4                                      |

#### EXAMPLE 7

(Comparative)

In order to impart long term storage stability to the concentrate of Example 6 an appropriate amount of Bentone 38 can be added. However this will increase the viscosity of the composition.

#### EXAMPLE 8

(Comparative)

5 A concentrate similar to example 6 can be made using, instead of the comminuted gel polymer, a bead polymer made by reverse phase bead polymerisation followed by azeotropic distillation and separation of the beads from the oil in which they were formed. This concentrate will generally require the addition of Bentone 38 or other dispersion promoter in order to impart storage stability to it.

#### EXAMPLE 9

10 A copolymer of 75 parts by weight acrylamide and 25 parts by weight of trimethyl 8-acryloxyethyl ammonium chloride was first prepared in a hydrocarbon liquid of boiling range 154°-168° C. (Shell SBP11) by conventional reverse phase polymerisation as follows. 15 287.4 gms of a 52.2% aqueous solution of acrylamide, 0.05 g of azo-bis-isobutyronitrile and 160.2 gms of water were mixed to form a solution whose pH was adjusted to 4.6 with sodium hydroxide solution (46% wt/wt) and then 71.0 gms of a 70.4% aqueous solution of trimethyl  $\beta$ -acryloxyethyl ammonium chloride was mixed in to form the aqueous monomer solution. An oil phase was prepared comprising 363.3 gms of SBP11, 14.2 gms at a 2 to 1 molar copolymer of stearyl methacrylate and methacrylic acid as suspension polymerisation stabiliser (as described in GB No. 1,482,515) and 7.8 gms Span 80.

20 The aqueous phase was homogenised with the oil phase and deoxygenated with nitrogen gas then polymerised by stirring in 1.5 mls of a 5% solution of sodium metabisulphite in water followed by a 1% solution of tertiary butyl hydroperoxide in SBP11 added at a rate of 0.25 mls per minute until polymerisation was complete.

25 The resulting aqueous polymer gel dispersion was azeotropically dehydrated under reduced pressure by recycling the SBP11. Part of the SBP11 was then distilled off resulting in an anhydrous polymer dispersion at a concentration of 40% polymer by weight in SBP11.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290

diluted with water to 0.1% by weight active size content and labelled K.

100 g.s.m. handsheets were prepared from a bleached sulphate/bleached birch stock containing 10% calcium carbonate loading on standard laboratory sheet making machine. Prior to sheet formation, the required amount of 0.1% emulsion labelled J was added to 600 mls of 1.0% consistency stock. After stirring, handsheets were prepared, pressed at 50 p.s.i. for 5 minutes prior to drying at 110° C. for 1 hour. After conditioning at room temperature, the degree of sizing was determined by the standard 1 minute cobb test.

Control sheets were prepared in the same manner as described above, but with emulsion K replacing emulsion J. The results are shown below:

| Emulsion | Dose Level of Alkenyl Succinic Anhydride Based on Dry Fibre and Filler | 1 Minute Cobb Value (g · m <sup>-2</sup> ) |
|----------|------------------------------------------------------------------------|--------------------------------------------|
| J        | 0.25%                                                                  | 22.1                                       |
| J        | 0.35%                                                                  | 16.4                                       |
| J        | 0.5%                                                                   | 13.7                                       |
| K        | 0.25%                                                                  | 27.2                                       |
| K        | 0.35%                                                                  | 20.1                                       |
| K        | 0.5%                                                                   | 15.6                                       |

We claim:

1. A concentrate composition suitable, upon dilution with water, for sizing cellulosic fibres and which comprises a substantially anhydrous dispersion of particles of water soluble cationic or anionic polyelectrolyte in a non-aqueous liquid comprising a reactive size and which contains water in an amount of 0 to 5% by weight of the total composition and which has been made by a process forming a dispersion in a water immiscible non-aqueous hydrophobic liquid of the polyelectrolyte particles while they are swollen by water, dehydrating the dispersion of polyelectrolyte particles swollen by water by azeotropic distillation until the dispersion is substantially anhydrous and dissolving the reactive size into the non-aqueous hydrophobic liquid of the resultant dehydrated dispersion, and in which the reactive size is selected from ketene dimer sizes and anhydride reactive sizes and the water soluble polyelectrolyte is selected from water soluble polymers of (a) cationic polymers formed from one or more ethylenically unsaturated monomers comprising a cationic ethylenically unsaturated monomer, (b) anionic polymers formed from one or more ethylenically unsaturated monomers comprising an ethylenically unsaturated carboxylic monomer or an ethylenically unsaturated sulfonic acid monomer, (c) polyamines, (d) dicyandiamide condensates and (e) polyimines.

2. A composition according to claim 1 containing at least one stabiliser for the aqueous polyelectrolyte particles in the hydrophobic liquid selected from water in oil emulsifiers and amphipathic polymeric dispersion stabilisers selected from oil soluble copolymers of one or more hydrophobic ethylenically unsaturated monomers with one or more hydrophilic ethylenically unsaturated monomers.

3. A composition according to claim 1 including amphipathic polymeric dispersion stabiliser selected from oil soluble copolymers of one or more hydrophobic ethylenically unsaturated monomers with one or more hydrophilic ethylenically unsaturated monomers.

4. A composition according to claim 1 in which the particles have a dry particle size of below 3  $\mu\text{m}$ .

5. A composition according to claim 1 in which the concentration of the reactive size is from 30 to 85% by weight of the composition and the weight ratio polyelectrolyte:size is from 1:1 to 1:10.

6. A composition according to claim 1 in which the polyelectrolyte is selected from polymers formed from at least one monomer selected from dialkylaminoalkyl (meth) acrylates and (meth) acrylamides and their acid addition salts and their quaternary ammonium salts, diallyl dialkyl ammonium chlorides, acrylic acid, methacrylic acid and 2-acrylamido-2-methyl propane sulfonic acid.

7. A composition according to claim 1 additionally including an oil-in-water emulsifier.

8. A composition according to claim 1 in which the said non-aqueous liquid comprises a solution of the size in the hydrophobic liquid and the ratio hydrophobic liquid:size by weight is 1:10 to 1:0.67.

9. A composition according to claim 1 in which the reactive size is a liquid reactive size and the said non-aqueous liquid consists essentially of the said liquid reactive size and the composition has been made by a process comprising the additional step of removing the said hydrophobic liquid after the addition of the size to the hydrophobic liquid.

10. A comparison according to claim 1 in which the dispersion of polyelectrolyte particles swollen by water in the hydrophobic liquid has been formed by reverse phase polymerisation of aqueous ethylenically unsaturated monomer while dispersed in the hydrophobic liquid.

11. A process of making a concentrate composition

suitable, upon dilution with water, for sizing cellulosic fibres and comprising forming a dispersion in a water immiscible non-aqueous hydrophobic liquid of particles of water soluble cationic or anionic polyelectrolyte particles swollen by water, dehydrating the dispersion of polyelectrolyte particles swollen by water by azeotropic distillation until the dispersion is substantially

anhydrous and dissolving into the hydrophobic liquid a reactive size, the resultant composition having a water content of from 0 to 5% by weight and in which the reactive size is selected from ketene dimer sizes and anhydride reactive sizes and the water soluble polyelectrolyte is selected from water soluble polymers of (a)

cationic polymers formed from one or more ethylenically unsaturated monomers comprising a cationic ethylenically unsaturated monomer, (b) anionic polymers formed from one or more ethylenically unsaturated monomers comprising an ethylenically unsaturated carboxylic monomer or an ethylenically unsaturated sulfonic acid monomer, (c) polyamines, (d) dicyandiamide condensates and (e) polyimines.

12. A method according to claim 11 in which the dispersion in the hydrophobic liquid of the polyelectrolyte particles swollen by water is formed in the presence of at least one stabiliser selected from water in oil emulsifiers and amphipathic polymeric dispersion stabilisers selected from oil soluble copolymers of one or more hydrophobic ethylenically unsaturated monomers with one or more hydrophilic ethylenically unsaturated monomers.

13. A method according to claim 11 in which the polyelectrolyte particles are stabilised in the dispersion by amphipathic polymeric dispersion stabiliser selected from oil soluble copolymers of one or more hydrophobic ethylenically unsaturated monomers with one or more hydrophilic ethylenically unsaturated monomers.

14. A method according to claim 11 in which the polyelectrolyte particles in the composition have a dry particle size below 3  $\mu\text{m}$ .

15. A method according to claim 11 in which the reactive size is a liquid size and the hydrophobic liquid is removed after the addition of the liquid size to the hydrophobic liquid.

16. A method according to claim 11 in which the dispersion in the hydrophobic liquid of the polyelectro-

lyte particles swollen by water is formed by dispersing an aqueous solution of the polyelectrolyte into the hydrophobic liquid.

17. A method according to claim 11 in which the dispersion in hydrophobic liquid of the polyelectrolyte particles swollen by water is formed by reverse phase polymerisation of aqueous ethylenically unsaturated monomer while dispersed in the hydrophobic liquid.

\* \* \* \* \*

10

15

20

25

30

35

40

45

50

55

60

65